

Jan. 31, 1950

P. A. JENNINGS  
HIGH-TEMPERATURE ARTICLE

2,496,246

Filed May 5, 1948

INFLUENCE OF SILICON CONTENT OF CHROMIUM-  
NICKEL-COBALT STAINLESS STEEL ON CORROSION  
RESISTANCE IN MOLTEN LEAD OXIDE.

SAMPLES OF 20% CHROMIUM - 15%  
NICKEL - 15% COBALT STAINLESS OF  
DIFFERING SILICON CONTENTS

TEMPERATURE - 1675° F  
FOR ONE HOUR  
SPECIMENS FLOATING



INVENTOR.  
PAUL A. JENNINGS  
BY *John H. Joyant*  
HIS ATTORNEY

## UNITED STATES PATENT OFFICE

2,496,246

## HIGH-TEMPERATURE ARTICLE

Paul A. Jennings, Baltimore, Md., assignor to  
Armco Steel Corporation, a corporation of Ohio

Application May 5, 1948, Serial No. 25,109

7 Claims. (Cl. 75—128)

1

This invention relates to high temperature stainless steel articles, especially to articles in the form of valves, valve parts and other internal combustion engine components intended for use while hot in corrosive atmospheres.

An object of my invention is the provision of strong, tough and durable austenitic stainless steel valves and valve parts for high temperature use, which offer substantial resistance to corrosion in the heated condition in atmospheres such as those containing the combustion products of so-called anti-knock gasoline of the tetra-ethyl lead variety.

A further object of my invention is that of providing high temperature stainless steel valves, valve parts, and any of a host of other internal combustion engine components, which in view of the excellent properties of the particular steel employed achieve highly satisfactory functions in such fields as passenger car, truck, aircraft, Diesel and marine vessel use.

Other objects in part will be obvious and in part pointed out more fully hereinafter.

The invention accordingly consists in the combination of elements, composition of materials and features of products, and in the relation of each of the same to one or more of the others as described herein, the scope of the application of which is indicated in the following claims.

The single figure of the accompanying drawing is a graph illustrating certain properties of steels, some of which fall within the scope of the present invention.

As conducive to a clearer understanding of certain features of my invention, it may be noted at this point that a great variety of heretofore known valves and valve parts intended for use as operating components of internal combustion engines or the like have become obsolete for such reasons as increased engine temperatures incident to greater engine power and speed. In average passenger cars, for example, the temperatures encountered by the valves frequently are as high as 700° F. or more at the fuel intake position, and as high as 1100° F. to 1450° F. or more at the exhaust position. These temperatures ordinarily are even higher in truck, bus, marine vessel or aircraft engines, especially in the region where the exhaust valves operate.

In most instances, low-alloy steel valves today are unsatisfactory in internal combustion engines, and this is especially so on the exhaust side of these engines. The valves usually burn or warp very quickly at the high operating temperatures, thus impairing engine efficiency and requiring

10 frequent replacement. While hot, the working parts commonly develop heat oxide scale, which detrimentally affects proper seating. In turn, failure to seat allows leakage or blow-by of the hot gases, thus increasing the valve temperature and burning away of the metal. An example of this type valve is one containing about 0.45% carbon, 8.50% chromium, 3.25% silicon, and the remainder substantially all iron.

15 A great number of the low-alloy steel valves have a low hot hardness value, and thus often are susceptible to deformation while hot as under the pounding effects of operation. Many of the products too are highly susceptible to creep at elevated temperatures and, accordingly, introduce injurious effects by appreciable changes in dimension by stretch. Also, most of the low-alloy steel valves are extremely susceptible to active corrosive attack by leaded fuels and particularly by the hot combustion products of these fuels. Additionally, a great majority of relatively high-alloy steel valves and parts likewise suffer great detriment and rapid deterioration when exposed to the combustion products of leaded fuels.

20 Quite some few valves and other internal combustion engine parts made of stainless steel have heretofore been introduced for better serving present-day needs. Some of these are of ferritic grade steel. Others are martensitic. In some, there is a high-silicon content and, as a result, they enjoy adequate scaling resistance. Unfortunately, however, the valves usually have poor resistance to lead compounds and are decidedly inferior in matters of hot hardness and stretch resistance under operating conditions, as will be appreciated more fully hereinafter.

25 There are other valves in the prior art among which are those of austenitic chromium-nickel stainless steel grade. The amounts of silicon in the conventional austenitic steel products ranges from about 0.50% to 4.0% or more. In general, the austenitic stainless steel valves have a more favorable lattice structure for resisting stress-rupture and creep at elevated temperatures than do the ferritic or martensitic products. It is also true that the relatively high alloy content of the chromium-nickel austenitic steels favors resistance to scaling from heat at engine temperatures. A further advantage often arising from austenitic steel valve products is their freedom from phase transformation and, in this respect, freedom from volume changes and any resulting tendencies such as warping, sticking or cracking during the heating and cooling cycles brought about by the heat engine and its operation. Many valves of this

character in the prior art, however, leave much to be desired of resistance to corrosive attack by lead compounds. There are many others which, despite the general merits of austenitic steels, fall on the inferior side with respect to hot hardness and resistance to creep.

An outstanding object of my invention accordingly is the provision of high-temperature, heat-resistant, corrosion-resistant stainless steel valves, valve parts, and other internal combustion engine components having substantial strength at elevated temperatures of use including resistance to creep, which are substantially free of phase transformation, are hot hard, and efficiently and reliably resist oxidation in the presence of heat and leaded fuel combustion products.

Referring now more particularly to the practice of my invention, I provide low-silicon, austenitic chromium-nickel-cobalt stainless steel high temperature products, as for example internal combustion engine intake or exhaust poppet valves, valve stems or heads, seats, balls, plungers, cores and springs, valve or cylinder claddings, linings or surfacing, or any of a host of other internal combustion engine components made of the steel. My products advantageously include about 0.05% to 1.5% carbon, from 12% to 25% chromium, 2% to 25% nickel, from 3% to 30% cobalt, and amounts of this element approximating 15% being preferred, from very small quantities up to about 0.20% silicon, and the remainder substantially all iron. By keeping an appreciable cobalt content in the steel, and the silicon content below about the 0.20% figure, I find sharp improvement in the resistance of the steel products to corrosion and attack by products of combustion resulting from the burning of leaded fuel. At about 0.10% silicon and on down substantially to zero per cent, this improvement is even more pronounced. The smaller quantities of silicon accordingly are usually preferred.

The cobalt addition importantly dispels an adverse effect of nickel on corrosion resistance in the presence of hot lead compounds. In being an austenite-former, the cobalt assists the maintenance of an austenitic balance of the steel. Also, the element, in the amounts employed, improves the hot hardness and high temperature stretch resistance of the steel products. On occasions, I use nitrogen in amounts up to about 0.30% as a substitute for an equivalent amount of carbon, nickel or cobalt in the steel. The nitrogen thus serves as an austenite-former. It also tends to increase the metal hot hardness a small degree.

The element manganese in my high temperature chromium-nickel-cobalt stainless steel products, preferably ranges from substantially zero in amount up to about 2%. The relatively large quantities within this range conveniently serve as a partial substitute for such austenite-forming elements as cobalt and nickel, thus to maintain the austenitic balance. There are occasions too where my stainless steel products include in the alloy composition thereof, as for special purposes, one or more such elements as molybdenum, titanium, columbium, tungsten, vanadium, copper, tantalum, aluminum, zirconium, or the like, ranging from quite small amounts to substantial amounts not inconsistent with properties desired.

The stainless steel valves, valve parts, and other internal combustion engine components which I provide have a phosphorus content pref-

erably below about 0.04%, and a sulphur content which amounts to less than 0.04%, or even as much as 0.5% or more. The larger quantities of sulphur, and especially those between about 0.15% to 0.50%, contribute to the effect of the cobalt and the low-silicon content in promoting resistance to attack by the combustion products of leaded gasolines and the like. The larger quantities of sulphur, say those much beyond 0.50% often introduce hot working difficulties with certain of the austenitic steels which I employ; also, the rate of improvement in resistance to corrosion by lead oxide usually decreases for these greater amounts.

My internal combustion engine valve products and the like, in containing chromium, nickel, cobalt and the very small quantities of silicon below about 0.20% have excellent heat resistance and resistance to oxidation at the high temperatures of operation. Also, the presence of cobalt and the restriction of silicon to the critically small amounts indicated importantly contribute to corrosion-resistance of the products in the combustion products of leaded fuels, as where the stainless steel takes the form of an exhaust valve or part exposed to aircraft, truck or passenger car anti-knock fuel exhaust gases. My stainless steel valves and other components of the steel, where made for purposes of operation under stress at high temperatures are resistant to creep. The metal is hot hard and strong, and resists scour and abrasion while heated. By virtue of the austenitic quality of the steel, my valve products suffer substantially no phase transformation during heating and cooling cycles, and, accordingly, are free of volume changes and difficulties often following upon change of phase. The valves resist scaling, warping and cracking at full temperature and upon being cooled and re-heated.

In the accompanying drawing, the approximate effect of different amounts of silicon on corrosion-resistance of 20% chromium, 15% nickel, 15% cobalt stainless steel in molten lead oxide is graphically illustrated. The carbon content of the several steel compositions concerned, is anywhere from about 0.05% to 0.10%, manganese about 0.5%, and sulphur and phosphorus each less than about 0.04%. Thus, the curve in the drawing is directed to steels which contain chromium, nickel, cobalt, manganese, sulphur and phosphorus in substantially the constant amounts noted, but each of the steels contains a different quantity of silicon as indicated below in the table, the remainder being substantially all iron. In this table, as in the accompanying drawing, the influence of silicon content on resistance in molten lead oxide for each steel is given in terms of grams weight loss per square decimeter per hour, for a corresponding temperature of 1675° F. of the molten lead oxide.

#### TABLE

65 *Influence of silicon on corrosion-resistance of certain chromium-nickel-cobalt stainless steels*

| Steel | Per Cent<br>Silicon | Weight Loss,<br>Gms. Per<br>Sq. Dc.<br>Per Hour |
|-------|---------------------|-------------------------------------------------|
| A     | 0.08                | 1.67                                            |
| B     | 0.19                | 3.53                                            |
| C     | 0.41                | 15.85                                           |
| D     | 0.79                | 17.24                                           |

It will be observed that the Steels A and B are steels falling within the scope of the present invention, the silicon content being sufficiently low, while the Steels C and D have a high silicon content and, accordingly, are not here claimed. In both the table and the graph, it is clear that by lowering the silicon content of the Steel C down to around 0.20%, as to the amount in the Steel B, a sharp improvement occurs in the resistance to lead oxide corrosion.

Thus it will be seen that in this invention there are provided a wide variety of low-silicon austenitic chromium-nickel-cobalt stainless steel articles and products, in which the various objects noted hereinbefore together with many thoroughly practical advantages are successfully achieved. It will be noted that the products are well suited for resisting corrosion in the presence of combustion products of leaded fuels.

While certain of the steels which I provide take the form of internal combustion engine components, it will be understood that certain advantages of the invention are had with other products of the low-silicon steel, among which are high-temperature gas turbine nozzles, turbine parts adjacent to the nozzle, and any of a number of supercharger components.

As many possible embodiments may be made of my invention, and as many changes may be made in the embodiment hereinbefore set forth, it will be understood that all matter described herein is to be interpreted as illustrative and not as a limitation.

I claim:

1. Stainless steel having great hardness at high temperatures and low stretch in combination with substantial resistance to corrosion in the presence of leaded fuel combustion products, and containing about 0.05% to 1.5% carbon, 12% to 25% chromium, from 2% to 25% nickel, 3% to 30% cobalt, all in such proportions as to assure a substantially fully austenitic structure, silicon not exceeding about 0.20%, and the remainder substantially all iron.

2. Stainless steel having great hardness at high temperatures and low stretch in combination with substantial resistance to corrosion in the presence of leaded fuel combustion products, and containing about 0.05% to 1.5% carbon, 12% to 25% chromium, from 2% to 25% nickel, 3% to 30% cobalt, all in such proportions as to assure a substantially fully austenitic structure, silicon not exceeding about 0.10%, and the remainder substantially all iron.

3. Stainless steel having great hardness at high temperatures and low stretch in combination with substantial resistance to corrosion in the presence of leaded fuel combustion products, and containing about 0.05% to 1.5% carbon, 12% to 25% chromium, from 2% to 25% nickel, 3% to 30% cobalt, all in such proportions as to assure a

substantially fully austenitic structure, 0.15% to 0.50% sulphur, phosphorus not exceeding 0.04%, silicon not exceeding about 0.20%, and the remainder substantially all iron.

5. Austenitic stainless steel internal combustion engine valves having great hardness at high temperatures and low stretch in combination with substantial resistance to corrosion in the presence of leaded fuel combustion products, and containing about 0.05% to 1.5% carbon, 12% to 25% chromium, from 2% to 25% nickel, 3% to 30% cobalt, silicon not exceeding 0.20%, up to 0.50% sulphur, phosphorus not exceeding 0.04%, and the remainder substantially all iron.

10. Austenitic stainless steel internal combustion engine valves having great hardness at high temperatures and low stretch in combination with substantial resistance to corrosion in the presence of leaded fuel combustion products, and containing about 0.05% to 1.5% carbon, 12% to 25% chromium, from 2% to 25% nickel, 3% to 30% cobalt, silicon not exceeding 0.20%, up to 2% manganese, and the remainder substantially all iron.

15. Austenitic stainless steel internal combustion engine valves having great hardness at high temperatures and low stretch in combination with substantial resistance to corrosion in the presence of leaded fuel combustion products, and containing about 0.05% to 1.5% carbon, 12% to 25% chromium, from 2% to 25% nickel, 3% to 30% cobalt, silicon not exceeding 0.20%, up to 2% manganese, and the remainder substantially all iron.

20. Austenitic stainless steel containing at least about 0.05% to 1.5% carbon, about 20% chromium, approximately 15% nickel, about 15% cobalt, silicon not exceeding about 0.20%, and the remainder substantially all iron.

25. Austenitic stainless steel internal combustion engine valves, containing about 0.05% to 1.5% carbon, about 20% chromium, approximately 15% nickel, about 15% cobalt, silicon not exceeding about 0.10%, and the remainder substantially all iron.

PAUL A. JENNINGS.

#### REFERENCES CITED

40. The following references are of record in the file of this patent:

#### UNITED STATES PATENTS

| Number       | Name          | Date          |
|--------------|---------------|---------------|
| 45 1,150,113 | Haynes        | Aug. 17, 1915 |
| 1,190,562    | Henderson     | July 11, 1916 |
| 1,522,813    | Etchells      | Jan. 13, 1925 |
| 2,163,561    | Payson et al. | June 20, 1939 |
| 50 2,397,034 | Mohling       | Mar. 19, 1946 |

#### FOREIGN PATENTS

| Number     | Country | Date          |
|------------|---------|---------------|
| 55 562,102 | France  | Nov. 5, 1923  |
| 653,900    | France  | Mar. 28, 1929 |

#### OTHER REFERENCES

Metals Handbook, 1939 edition, page 47. Published by the American Society for Metals, Cleveland, Ohio.

60. Chemical Abstracts, volume 28, column 3374. Published by The American Chemical Society at Easton, Pa.